

## UNITED STATES PATENT OFFICE

2,399,817

## MINERAL OIL

Ronald E. Meyer, Woodbury, N. J., assignor to  
Socony-Vacuum Oil Company, Incorporated, a  
corporation of New York

No Drawing. Application October 12, 1943,  
Serial No. 505,965

14 Claims. (Cl. 252—52)

This invention has to do with lubricating oils of improved viscosity characteristics and more specifically has to do with lubricating oils enhanced by the incorporation therein of small amounts of oil-soluble polymers.

As is well known to those familiar with the art, the viscosity of an oil fraction varies considerably with temperature change. It is this characteristic that has limited the utility of certain oils to only those operations where temperature change is relatively small. The naphthenic oils are notable in this regard inasmuch as the viscosity change over a temperature range of 100° F., for example, is extreme. On the other hand, paraffinic oils suffer a substantially smaller change over the same temperature range. This characteristic has generally been expressed in the art as the "viscosity index (V. I.)" which is the rate of change of viscosity of naphthenic and paraffinic oil fractions with temperature change and is described in detail by Dean and Davis in the *Chem. & Met. Eng.* 36, 618 (1929).

Inasmuch as many of the hitherto useful lubricating oil fractions have been found to be unsuitable for use in several present day operations which require oils having relatively high viscosity indexes, a demand has arisen for new lubricants. In general, the new lubricants which have been developed can be divided into two categories: synthetic lubricants, and lubricating oil fractions enhanced by small amounts of improving agents which have been termed "viscosity index improving agents." This invention is directed to lubricants of the latter category and, more particularly, is predicated upon the discovery of a new class of viscosity index improving agents.

The improving agents which we have found to impart substantial improvement in viscosity characteristics to lubricating oil fractions, are oil-soluble, neutral co-polymers obtained by reacting diolefins with carbonyl compounds selected from the group consisting of unsaturated ketones and aldehydes, in the presence of various catalysts.

While, in general, all diolefins may be used in the production of the co-polymers defined above, conjugated diolefins are preferred and, of this group, butadiene is particularly preferred.

The carbonyl compounds used herein are, as aforesaid, unsaturated aliphatic ketones and aldehydes. These compounds may also be defined as decarboxylation products of aliphatic, cycloaliphatic and aliphatic-cycloaliphatic acids. For example, when oleic acid is decarboxylated, the

predominant product obtained thereby is dioleyl ketone; and, similarly, when a naphthenic acid is decarboxylated, the predominant product is an unsaturated dinaphthenyl ketone. Correspondingly, if a mixture of naphthenic acid and formic acid is decarboxylated, the product is predominantly aldehydes. While the foregoing decarboxylation products may be used in the pure state in the reaction with a diolefin, crude decarboxylation products may also be used.

Of the foregoing compounds, however, the unsaturated ketones are preferred, and of this group, dioleyl and unsaturated naphthenyl ketones are particularly preferred.

15 Co-polymers of unsaturated carbonyl compounds and diolefins are oil-soluble and neutral, and possess different properties depending upon the method of polymerization resorted to for their preparation. For example, soft, plastic, rubber-like (elastomeric), oil-soluble, neutral co-polymers are preferably prepared by using from about 40 to about 60 mol per cent of the unsaturated carbonyl compound in the reaction, and temperatures in the range of from about 150° C. to about 300° C. Catalysts of the 20 peroxide type are preferably employed in preparing such resins. Illustrative of such catalysts are benzoyl peroxide and sodium perborate. In order to prepare hard, brittle, transparent-varnish type resins, it is preferred that the unsaturated carbonyl compound should be present in the reaction mixture in the amount of from about 30 to about 75 mol per cent or more and that 25 temperatures of the order of —40° C. to about +25° C. should be used. The catalysts which are preferred for the preparation of this latter type of co-polymer are of the metal halide type, for example,  $AlCl_3$ ,  $BF_3$ ,  $SnCl_4$ , etc. In each of 30 these illustrative methods of preparation, organic solvents such as ethylene di- or tetra-40 chloride may be present.

In order to more fully illustrate the co-polymers contemplated herein as mineral oil improving agents, the preparations of several preferred 45 polymers are described below:

## RUBBER-LIKE CO-POLYMERS

## EXAMPLE 1

50 Co-polymer of unsaturated naphthenyl ketone and butadiene

(a) Preparation of unsaturated naphthenyl ketone:

A naphthenic acid, having a boiling range from about 150° C. to about 300° C., was passed over

calcium oxide which was contained in a heated muffle furnace, at a rate of about 25 to about 40 grams per hour and at a temperature of about 300 to 475° C. The product obtained by this treatment is an unsaturated naphthyl ketone boiling from about 100° C. to about 350° C.

(b) Preparation of co-polymer of butadiene and (a):

One hundred and fifty grams of the unsaturated naphthyl ketone prepared as described in (a), 174 grams of butadiene and 10 grams of benzoyl peroxide were charged to a 500 cc. steel shaker bomb. The temperature of the bomb was held at about 190° C. to about 260° C. for nine hours during which time the polymerization occurred. The reaction product was then diluted with benzol, filtered, washed with water and distilled to a maximum temperature of 200° C. at 200 mm. The co-polymer obtained by this treatment was neutral, viscous, transparent, rubber-like and oil-soluble, and had a molecular weight of 1652. This product is identified herein as co-polymer I.

#### EXAMPLE 2

##### *Co-polymer of oleyl ketone and butadiene*

A one-liter, three necked flask equipped with a motor stirrer, a thermometer and a 500 cc. dropping funnel was cooled to -40° C. Then 46 grams of oleyl ketone and 92 grams of butadiene were added to the flask. A quantity of 4 grams of anhydrous aluminum chloride which had previously been dissolved in 200 cc. of ethylene dichloride was placed in the dropping funnel and added to the mixture in the flask, drop by drop, over a 1½ hour period. When the addition had been completed, the temperature was allowed to rise to about 25° C. and stirring was continued for 16 hours. The reaction product was then filtered through super Filtral clay and the filtrate was distilled to a maximum temperature of 230° C. at 760 mm. The co-polymer thus obtained, co-polymer II, was a soft, plastic, transparent, rubber-like, oil-soluble, neutral resin.

#### RESINOUS CO-POLYMERS

#### EXAMPLE 3

##### *Co-polymers of unsaturated naphthyl ketone and butadiene*

A one-liter, three-necked flask, equipped with a motor stirrer, a thermometer and a long glass tube extending to the bottom of the flask, was cooled to about -20° C. Eighty-five grams of unsaturated naphthyl ketone prepared as described in (a), 28 grams of butadiene and 200 cc. of ethylene dichloride were then added to the flask. The lowest temperature at which the unsaturated naphthyl ketone remained in solution with the ethylene dichloride and butadiene was about -20° C. Boron trifluoride was then very slowly bubbled into the reaction mixture and the temperature was maintained at about -5° C. for about fifteen minutes. There was then a vigorous reaction with the temperature rapidly rising to about +5° C. The temperature was allowed to rise to 18° C. where it was held constant for one hour. The reaction product was diluted with benzol, filtered through 50 grams of Super Filtral clay and distilled to a maximum temperature of 230° C. at 5 mm. The co-polymer obtained was a very hard, brittle, transparent, neutral resin of the varnish type (oil soluble) having a molecular weight of 1092, and is identified herein as co-polymer III.

#### EXAMPLE 4

##### *Co-polymer of oleyl ketone and butadiene*

A one-liter, three necked flask equipped as described in Example 3 was cooled to -35° C. and 100 grams of oleyl ketone, 30 grams of butadiene and 200 cc. of ethylene di-chloride were then added to the flask. After cooling the reaction mixture to -35° C., boron trifluoride was bubbled slowly into the mixture. The temperature remained at -35° C. for fifteen minutes and then began to rise very slowly to 25° C. where it was held constant for 1½ hours with constant stirring. The reaction product was filtered through Super Filtral clay. In this way a soft, plastic, transparent, oil-soluble, neutral resin having a molecular weight of 838 was obtained. This product is referred to herein as co-polymer IV.

The effectiveness of the co-polymers of the type contemplated herein in improving the viscosity index of lubricating oils is demonstrated herein by viscosity data obtained on a lubricating oil and on oil blends of the same oil containing small amounts of co-polymer I. The oil used was a viscous mineral oil of the lubricant type and the data was obtained in the conventional manner from the kinematic viscosities of the oil and of the oil blends at 100° F. and at 210° F. The results are shown below in the table.

Table

| Improving agent | Conc. by wt., per cent | Kinematic viscosity |         | V. I. |
|-----------------|------------------------|---------------------|---------|-------|
|                 |                        | 100° F.             | 210° F. |       |
| None            |                        | 20.56               | 4.72    | 76.7  |
| Co-polymer I    | 2                      | 35.25               | 5.61    | 106.9 |
| Do              | 1                      | 32.51               | 5.16    | 94.4  |
| Do              | 0.5                    | 31.22               | 4.98    | 88.8  |

As will be apparent from the foregoing data, substantial improvement in the viscosity characteristics of lubricating oils is imparted by small amounts of the co-polymers contemplated herein. In general amounts of from about 0.1% to about 5% may be used, although appreciable improvement is obtained with amounts from about 0.25% to about 2.0%.

It is to be understood that this invention is not limited to the foregoing illustrative reactants, reaction conditions and co-polymers, but is to be construed in accordance with the broad disclosure set forth hereinabove. The invention, therefore, is to be interpreted as coming within the spirit of the appended claims.

I claim:

1. An improved mineral oil composition comprising a mineral oil fraction having in admixture therewith a minor proportion, sufficient to improve the viscosity characteristics of said oil fraction, of an oil-soluble, neutral co-polymer of a diolefin and a carbonyl compound selected from the group consisting of an unsaturated aliphatic ketone and an aliphatic aldehyde.
2. An improved mineral oil composition comprising a mineral oil fraction having in admixture therewith a minor proportion, from about 0.1 per cent to about 5.0 per cent, of an oil-soluble, neutral co-polymer of a diolefin and a carbonyl compound selected from the group consisting of an unsaturated aliphatic ketone and an aliphatic aldehyde.
3. An improved mineral oil composition comprising a mineral oil fraction having in admixture therewith a minor proportion, sufficient to im-

prove the viscosity characteristics of said oil fraction, of an oil-soluble, neutral co-polymer of a diolefin and an unsaturated aliphatic ketone.

4. An improved mineral oil composition comprising a mineral oil fraction having in admixture therewith a minor proportion, sufficient to improve the viscosity characteristics of said oil fraction, of an oil-soluble, neutral co-polymer of a conjugated diolefin and an unsaturated aliphatic ketone.

5. An improved mineral oil composition comprising a mineral oil fraction having in admixture therewith a minor proportion, sufficient to improve the viscosity characteristics of said oil fraction, of an oil-soluble, neutral co-polymer of butadiene and an unsaturated aliphatic ketone.

6. An improved mineral oil composition comprising a mineral oil fraction having in admixture therewith a minor proportion, sufficient to improve the viscosity characteristics of said oil fraction, of an oil-soluble, neutral co-polymer of dioleyl ketone and butadiene.

7. An improved mineral oil composition comprising a mineral oil fraction having in admixture therewith a minor proportion, sufficient to improve the viscosity characteristics of said oil fraction, of an oil-soluble, neutral co-polymer of an unsaturated naphthenic ketone and butadiene.

8. An improved mineral oil composition comprising a mineral oil fraction having in admixture therewith a minor proportion, sufficient to improve the viscosity characteristics of said oil fraction, of an oil-soluble, elastomeric, neutral co-polymer obtained by the reaction of an unsaturated aliphatic ketone and a diolefin.

9. An improved mineral oil composition comprising a mineral oil fraction having in admixture therewith a minor proportion, sufficient to improve the viscosity characteristics of said oil

fraction, of an oil-soluble, resinous, neutral co-polymer obtained by the reaction of an unsaturated aliphatic ketone and a diolefin.

10. An improved mineral oil composition comprising a mineral oil fraction having in admixture therewith a minor proportion, sufficient to improve the viscosity characteristics of said oil fraction, of an oil-soluble, elastomeric, neutral co-polymer obtained by reaction of an unsaturated naphthenic ketone and butadiene.

11. An improved mineral oil composition comprising a mineral oil fraction having in admixture therewith a minor proportion, sufficient to improve the viscosity characteristics of said oil fraction, of an oil-soluble, resinous, neutral co-polymer obtained by reaction of an unsaturated naphthenic ketone and butadiene.

12. An improved mineral oil composition comprising a mineral oil fraction having in admixture therewith a minor proportion, sufficient to improve the viscosity characteristics of said oil fraction, of an oil-soluble, resinous, neutral co-polymer obtained by reaction of dioleyl ketone and butadiene.

13. An improved mineral oil composition comprising a mineral oil fraction having in admixture therewith a minor proportion, sufficient to improve the viscosity characteristics of said oil fraction, of an oil-soluble, neutral co-polymer of a diolefin and an aliphatic aldehyde.

14. An improved mineral oil composition comprising a mineral oil fraction having in admixture therewith a minor proportion, sufficient to improve the viscosity characteristics of said oil fraction, of an oil-soluble, neutral co-polymer of a diolefin and a decarboxylation product of an acid selected from the group consisting of aliphatic, cycloaliphatic and aliphatic-cycloaliphatic acids.

RONALD E. MEYER.